

1

3,539,512  
**POLYETHYLENE THICKENED GREASE  
CONTAINING AMIDES**

Raymond Rohde and Andrew E. Skeen, Bartlesville, Okla., assignors to Phillips Petroleum Company, a corporation of Delaware  
No Drawing. Filed Nov. 25, 1968, Ser. No. 778,818  
Int. Cl. C10m 5/22

U.S. Cl. 252—33.3

5 Claims

**ABSTRACT OF THE DISCLOSURE**

Greases exhibiting little tendency to bleed (separation of oil) are compounded from an oil, polyolefin thickener, amide compound, sulfur-nitrogen heterocyclic compounds, lead naphthalene, salts of dinonylnaphthalene sulfonate, octylated diphenylamines and lead dialkyldithiocarbamates.

This invention relates to lubricants and more particularly to bodied lubricants or greases.

A very common deficiency of lubricant greases is the tendency for oil to separate (bleed) therefrom especially if the greases are subjected to extreme temperature conditions. Excessive oil separation from lubricant greases is, of course, undesirable. For example, it is highly desirable that greases employed as automotive chassis lubricants exhibit very little tendency to bleed oil.

Accordingly, it is a principal object of this invention to provide grease compositions which exhibit very little tendency to bleed oil.

The low oil-bleeding greases of this invention are formulated from a lubricating oil thickened with a polyolefin to the consistency of a grease. The greases contain minor amounts of certain other components, the combination of which results in a grease which exhibits a remarkably low tendency to bleed oil.

Particularly preferred greases of this invention have the following composition:

| Grease components:                                    | Approximate range, weight percent |
|-------------------------------------------------------|-----------------------------------|
| (A) Base oil                                          | 67.0—95.9                         |
| (B) Polyolefin thickener                              | 1.0—20                            |
| (C) Amide                                             | 0.1—5                             |
| (D) Sulfur-nitrogen heterocyclic compound             | 0.5—1.5                           |
| (E) Lead naphthalene                                  | 1.0—3.0                           |
| (F) Alkali metal salt of dinonylnaphthalene sulfonate | 0.5—1.0                           |
| (G) Octylated diphenylamines                          | 0.5—1.0                           |
| (H) Lead dialkyldithiocarbamate                       | 0.5—1.5                           |

The base oil can be any oil of lubricating grade such as those customarily used in compounding greases. Thus, the lubricating oil base can be a mineral, vegetable or animal oil or mixtures thereof. It is preferred that at least a major amount of the lubricating base oil be mineral in origin and most preferably a refined oil having a viscosity of about 50 to 240 SUS at 210° F. Less viscous lubricating oils result in lighter greases while heavier greases can be prepared from more viscous type oils, for example an oil having a viscosity of about 70 to 240 SUS at 210° F. White mineral oil can be used to make non-staining greases which are particularly adapted for lubricating machinery in the textile and food industries. Paraffinic oils are preferred for the preparation of greases of low graininess.

The polyolefin thickeners employed in accordance with this invention are ethylene polymers having a density at 25° C. of at least 0.940 gram per cubic centimeter. Such

2

ethylene polymers are disclosed in U.S. Pat. No. 3,112,270 and the disclosure therein is incorporated by reference herein. The density of these polymers generally will not exceed 0.970 although more dense, for example, polymers having a density of 1.00, can be used. The ethylene polymers which are employed include not only the homopolymer, polyethylene, but also copolymers of ethylene with olefins of higher molecular weight, for example up to 8 carbon atoms per molecule, preferably containing no branching nearer the double bond than the 4-position. Examples of suitable comonomers include propylene, 1-butene, 2-butene, 1-pentene, 1-octene, 4-methyl-1-pentene, 4-ethyl-1-pentene, 4-methyl-1-hexene, 6-methyl-1-heptene, 4-ethyl-1-hexene and the like. The copolymers of ethylene with propylene or 1-butene are preferred and it is preferred that the polymers of ethylene be employed in fluff form. In general, ethylene makes up at least 95 weight percent of the copolymer. In forming such a polymer the monomer feed to the polymerization zone will ordinarily be at least 80 percent by weight ethylene. As the percent of ethylene in the copolymer is decreased the density of the polymer likewise is decreased so that the density limitation can be used as an indication of copolymer composition. In any event, the density of the copolymer or homopolymer employed will be at least 0.940. The amount of polymer employed to thicken the lubricating oil to produce the desired greases will depend upon the specific oil and polymer used and upon the desired hardness of the grease. Most often, the polymer concentration in the finished grease will be in the range of 7—15 weight percent.

The amide component (C) is an N-substituted- $\gamma$ -hydrocarboxylic acid amide or mixtures of such amides. These additives can be represented by the general formula:



wherein R represents either hydrogen or a methyl group, R<sup>1</sup> represents an aliphatic hydrocarbon radical (saturated or unsaturated) containing from 10 to 30 carbon atoms, for example, decyl, undecyl, undecylenyl, dodecyl, tridecyl, tetradecyl, cetyl, myristoleyl, pentadecyl, heptadecyl, hexadecenyl, octadecyl, octadecenyl, octadecadienyl, abietinyl, oleyl, elaidyl, octylbenzyl, eicosyl, triacontyl, and the like and combinations of such radicals; and wherein R<sup>2</sup> represents either hydrogen or alkyl group of from 1 to about 18 carbon atoms, for example, methyl, propyl, butyl, amyl, hexyl, nonyl, decyl, dodecyl, cetyl, octadecyl, and the like; and wherein the total number of carbon atoms constituting the groups in both R<sup>1</sup> and R<sup>2</sup> is a minimum of 10 and not more than about 40 carbon atoms.

The compounds characterized by the above formula and utilized in accordance with the present invention can be obtained by conventional methods such as the reaction of one mole of an organic primary amine, or mixtures of such amines, containing from 10 to about 30 carbon atoms with one mole of either gamma-butyrolactone or gamma-valerolactone at a temperature of about 80—95° C. The amines have the formula



wherein R<sup>1</sup> and R<sup>2</sup> have the values indicated above. Preferably, both R and R<sup>2</sup> are hydrogen and R<sup>1</sup> is formed from a mixture of saturated or unsaturated amine residues derived from naturally occurring fatty acids (by replacing the carboxyl group with a primary amino group) such as are obtained from coconut oil, soya oil, tallow, and the

## 3

like which are commercially available (for example, under the brand name of "Duomeens").

Grease component D is a 2-mercaptopbenzothiazole compound, an anti-rust agent conforming to the formula



wherein R³ is selected from hydrogen or from alkyl, aryl, or cycloalkyl radicals, or combinations of these such as aralkyl, or alkaryl, containing from 1 to about 12 carbon atoms per radical, and wherein the total of all the carbon atoms in all of the R³ radicals in the molecule will not exceed about 20. Some examples of suitable R³ groups are methyl, ethyl, propyl, isobutyl, benzyl, phenyl, cyclohexyl, dodecyl, paratolyl, 2-ethylhexyl, and the like, and mixtures thereof. R³ is preferably hydrogen.

Although the above-described substituted and unsubstituted 2-mercaptopbenzothiazole compounds can be used, it is sometimes preferred that they be utilized in the form of their amine salts. Consequently, the above mercapto compounds can be combined with an equivalent weight of a primary, secondary, or tertiary amine compound. Such amine compounds can be monoamines or polyamines and can contain from about 2 to about 30 carbon atoms per molecule, preferably from about 10 to about 24 carbon atoms per molecule. The preferred amines are those obtained from naturally occurring materials such as long chain organic acids derived from soya oil, coconut oil, tallow, and the like. Such "fatty" amines are commercially available (for example, under the brand name of Duomeens) and are prepared by conventional methods. The amine salt of the above mercapto compound is conventionally prepared merely by reacting equivalent quantities of these materials generally at elevated temperatures.

Component E is lead naphthenate. This is a commercially available material which is a derivative of naphthenic acids which are, in turn, derived from petroleum. This component imparts desirable extreme pressure properties to the composition. It is believed that these acids are produced in part by oxidation of certain readily oxidized cycloparaffins (naphthenes) during distillation or other petroleum-refining operations. Such acids dissolve in the aqueous caustic solutions used in refining. Lead naphthenate is produced merely by the addition of a lead salt to the aqueous sodium naphthenate solution. Thus, while the acid portion of these ingredients is a complex mixture, such a material, and its preparation, are well known in the petroleum art.

Component F of the grease composition is an alkali metal salt of a dinonylnaphthalene sulfonate corresponding to the formula



wherein M is an alkali metal and the C9H19 radicals are either branched or unbranched radicals. Such materials are commercially available as anti-rust agents and are conventionally prepared such as by the alkylation of naphthalene followed by sulfonation and neutralization. Sodium is the preferred metal.

Grease component G is one or more octylated diphenyl amines corresponding to the formula



wherein the C8H17 radical can be either branched or unbranched. These materials serve as anti-oxidants.

## 4

Grease component H, the inclusion of which is optional, is a lead dialkyldithiocarbamate having the formula



wherein each R⁴ is a branched or unbranched alkyl radical having from 1 to about 10 carbon atoms per radical. Thus, R⁴ radicals such as methyl, ethyl, isopropyl, isobutyl, amyl, octyl, nonyl, decyl, and the like can be present.

The soapless, low-bleeding greases of the present invention are compounded, in general, by conventional methods such as those taught in U.S. Pat. No. 3,112,270,

15 Thus, the solid ethylene polymer is dispersed in the lubricating oil which has been heated to about 325 to 450° F. and generally above 380° F. for a period of time required to form a satisfactory polymer-oil dispersion. Usually, the polymer is adequately dispersed within about 20 1 to 60 minutes. The amide additive, as well as other conventional grease additives, is blended in with the grease during this polymer dispersion operation. The mixture is then cooled to a temperature of about 200-250° F. and the grease components D, E, F, G and H blended therein.

25 In addition to the polymer dispersion and additive incorporation steps, the greases are generally milled to improve their properties. In this milling operation the polymer-oil-additive dispersion described above is cooled to a temperature between about 170 and 210° F. and subjected to severe agitation which produces substantial shearing in the mixture. Preferably the grease milling is carried out in a colloid mill operated at high speeds and with relatively close clearances. Such grease milling is conventional and known in the art.

30 35 The following are representative examples of greases prepared in accordance with this invention.

## Grease A: Wt. Percent

|    |                                                                 |       |
|----|-----------------------------------------------------------------|-------|
| 40 | Mineral lubricating oil 195 SUS at 210° F.)                     | 11.50 |
|    | Polyolefin thickener (density 0.95)                             | 11.50 |
|    | Reaction product of octadecylamine with $\gamma$ -butyrolactone | 2.50  |
| 45 | 2-mercaptopbenzothiazole                                        | 1.00  |
|    | Lead naphthenate                                                | 2.00  |
|    | Sodium salt of dinonylnaphthalene sulfonate                     | 0.75  |
|    | Mixture of octylated diphenylamines                             | 0.75  |
|    | Lead dipropyldithiocarbamate                                    | 0.50  |

## Grease B:

|    |                                                               |      |
|----|---------------------------------------------------------------|------|
|    | Mineral lubricating oil (150 SUS at 210° F.)                  | 85.0 |
| 55 | Polyolefin thickener (density 0.94)                           | 7.8  |
|    | Reaction product of N-decylamine with $\gamma$ -butyrolactone | 1.8  |
|    | 2-mercaptop-tetrapropylbenzothiazole                          | 0.6  |
| 60 | Lead naphthenate                                              | 1.5  |
|    | Sodium salt of dinonylnaphthalene sulfonate                   | 0.5  |
|    | Octylated diphenylamine                                       | 1.0  |
|    | Lead dioctyldithiocarbamate                                   | 1.0  |

## Grease C:

|    |                                                                                                                                              |       |
|----|----------------------------------------------------------------------------------------------------------------------------------------------|-------|
| 65 | Paraffinic lubricating oil (210 SUS at 210° F.)                                                                                              | 76.00 |
|    | Polyolefin thickener (density 0.954)                                                                                                         | 13.00 |
|    | Reaction product of 0.2 mole $\gamma$ -valerolactone and 0.2 mole of a mixture of aliphatic primary amines derived from soya oil fatty acids | 4.00  |
| 70 | 2-mercaptopbenzothiazole                                                                                                                     | 1.50  |
|    | Lead naphthenate                                                                                                                             | 3.00  |
|    | Potassium salt of dinonylnaphthalene sulfonate                                                                                               | 0.50  |
|    | Octylated diphenylamine                                                                                                                      | 0.50  |
| 75 | Lead methylhexyldithiocarbamate                                                                                                              | 1.50  |

## Grease D:

|                                                                                                                                                                                            |       |
|--------------------------------------------------------------------------------------------------------------------------------------------------------------------------------------------|-------|
| Naphthenic lubricating oil (95 SUS at 210° F.)                                                                                                                                             | 78.15 |
| Polyolefin thickener (density 0.96)                                                                                                                                                        | 13.20 |
| Reaction product of 86.1 grams of $\gamma$ -butyrolactone with 274 grams of a mixture of amines: Hexadecylamine 10%, octadecylamine 10%, octadecenylamine 35%, and octadecadienylamine 45% | 5     |
| 2-mercaptop-tetrabutylbenzothiazole                                                                                                                                                        | 3.20  |
| Lead naphthenate                                                                                                                                                                           | 1.20  |
| Sodium salt of dinonylnaphthalene sulfonate                                                                                                                                                | 10    |
| Octylated diphenylamine                                                                                                                                                                    | 0.75  |
| Lead diisobutylthiocarbamate                                                                                                                                                               | 0.60  |
|                                                                                                                                                                                            | 1.90  |
|                                                                                                                                                                                            | 1.00  |
|                                                                                                                                                                                            | 15    |

The low bleeding characteristics of greases compounded in accordance with the present invention are readily apparent by the bleed test results obtained in comparison with other grease compositions. Using test method ASTM D 1742-64, Greases E and F, (particularly preferred greases of this invention) was compared with Greases G, H and I, which greases are not in accordance with the invention. Greases E, F, G, H and I were prepared by first dispersing the polyethylene thickener into the oil by simple mixing at a temperature of 320° F. After the polyethylene was dispersed the amide was incorporated into the mixture. The mixture was then cooled to a temperature of about 225° F. and the other additives, if any, were added. The mixture was then further cooled to about 190° F. and milled by passage through a Charlotte colloid mill. The entrained air was removed from the grease while it was hot, with the aid of a vacuum pump. Each of these greases had essentially the same hardness, being in the range of an NLGI Grade 2 grease. The composition of Greases E, F, G, H and I are set forth below:

|                                                                                                                                     | Grease E, wt. percent | Grease F, wt. percent | Grease G, wt. percent | Grease H, wt. percent | Grease I, wt. percent |
|-------------------------------------------------------------------------------------------------------------------------------------|-----------------------|-----------------------|-----------------------|-----------------------|-----------------------|
| Refined lubricating oil (110 SUS at 210° F.) derived from Mid-Continent crude                                                       | 85.0                  | 86.0                  | 91.0                  | 90.0                  | 87.0                  |
| Polyethylene (density ~0.960, melt index ~5.0)                                                                                      | 9.0                   | 9.0                   | 9.0                   | 9.0                   | 9.0                   |
| N-coco- $\gamma$ -hydroxybutyramide (Butoxyne 160, General Aniline and Film Corp.)                                                  | 1.0                   | 1.0                   | 1.0                   | 1.0                   | -----                 |
| Unsubstituted 2-mercaptopbenzothiazole in the form of a salt with a high molecular weight amine (Vanlube 601, R. T. Vanderbilt Co.) | 1.0                   | 1.0                   | -----                 | -----                 | 1.0                   |
| Lead naphthenate                                                                                                                    | 2.0                   | 2.0                   | -----                 | -----                 | 2.0                   |
| Sodium salt of dinonylnaphthalene sulfonate                                                                                         | 0.5                   | 0.5                   | -----                 | -----                 | 0.5                   |
| Mixture of octylated diphenylamines (Vanlube SL, R. T. Vanderbilt Co.)                                                              | 0.5                   | 0.5                   | -----                 | -----                 | 0.5                   |
| Lead diisobutylthiocarbamate (Vanlube 71)                                                                                           | 1.0                   | 1                     | 3                     | >20                   | 10                    |
| Oil separation after 96 hours, ml                                                                                                   |                       |                       |                       |                       | 15                    |

These data clearly illustrate the surprising results obtained from the invention Greases E and F. The combination of components in these grease formulations results in an unexpected decrease in oil bleeding. Such improved results are not possible by merely incorporating a random choice of any of the conventionally known grease additives. Indeed, the addition of some commonly used grease additives substantially increases oil bleeding. The grease compositions of the present invention are valuable in that the greases have an excellent balance of performance properties in addition to the low bleeding characteristic.

The Butoxyne 160 in Greases E, F and H is a product formed by reacting  $\gamma$ -butyrolactone with a mixture of saturated and unsaturated primary amines derived from coconut oil.

Those modifications and equivalents which fall within the spirit of the invention are to be considered a part thereof.

We claim:

1. A lubricant comprising a major amount of lubricating oil thickened with an ethylene polymer having a density of at least 0.940 gram per cubic centimeter at 25° C. and minor effective amounts of additives (C), (D), (E), (F), (G) and (H) wherein

70  
75

additive (C) is an amide of the formula



wherein

R is hydrogen or methyl,

R<sup>1</sup> is an aliphatic hydrocarbon radical containing from 10 to 30 carbon atoms, and

R<sup>2</sup> is hydrogen or an alkyl group of from 1 to 18 carbon atoms and wherein the total number of carbon atoms in R<sup>1</sup> and R<sup>2</sup> is in the range from 10 to 40;

additive (D) is a 2-mercaptobenzothiazole compound conforming to the formula



wherein R<sup>3</sup> is selected from hydrogen or from alkyl, aryl, or cycloalkyl radicals, or combinations thereof, containing from 1 to about 12 carbon atoms per radical, and wherein the total of all the carbon atoms in all of the R<sup>3</sup> radicals on the molecule will not exceed about 20;

additive (E) is lead naphthenate;

additive (F) is an alkali metal salt of a dinonylnaphthalene sulfonate corresponding to the formula



wherein M is an alkali metal and the C<sub>9</sub>H<sub>19</sub> radicals are either branched or unbranched radicals;

additive (G) is octylated diphenylamines corresponding to the formula



wherein the C<sub>8</sub>H<sub>17</sub> radical can be either branched or unbranched;

additive (H) is a lead dialkyldithiocarbamate.

2. A lubricant in accordance with claim 1, wherein additive (C) is employed in the lubricant in an amount of from 0.1 to 5% by weight,

additive (D) is employed in the lubricant in an amount of from 0.5 to 1.5% by weight,

additive (E) is employed in the lubricant in an amount of from 1.0 to 3.0% by weight,

additive (F) is employed in the lubricant in an amount of from 0.5 to 1.0% by weight,

additive (G) is employed in the lubricant in an amount of from 0.5 to 1.0% by weight.

additive (H) is employed in the lubricant in an amount of from 0.5 to 1.5% by weight.

3. A lubricant in accordance with claim 2 wherein

additive (C) is N-coco- $\gamma$ -hydroxybutyramide and additive (D) is 2-mercaptopbenzothiazole.

4. A thickened lubricant comprising:

about 85% by weight of a mineral lubricating oil,  
about 9.0% by weight of polyethylene having a density  
of about 0.960 gram per cubic centimeter at 25° C.,  
about 1.0% by weight of N-coco- $\gamma$ -hydroxybutyramide,  
about 1.0% by weight of a high molecular weight amine  
salt of 2-mercaptopbenzothiazole,  
about 2.0% by weight of lead naphthenate,  
about 0.5% by weight of the sodium salt of dinonyl-  
naphthalene sulfonate,  
about 0.5% by weight of an octylated diphenylamine,  
and  
about 1.0% by weight of lead diayldithiocarbamate. 15

5. A lubricant comprising a major amount of lubricating oil thickened with an ethylene polymer having a density of at least 0.940 gram per cubic centimeter at 25° C. and minor effective amounts of additives (C), (D), (E), (F) and (G) wherein

additive (C) is an amide of the formula



wherein R is hydrogen or methyl,

$\text{R}^1$  is an aliphatic hydrocarbon radical containing  
from 10 to 30 carbon atoms, and

$\text{R}^2$  is hydrogen or an alkyl group of from 1 to 18  
carbon atoms and wherein the total number of  
carbon atoms in  $\text{R}^1$  and  $\text{R}^2$  is in the range from  
10 to 40;

additive (D) is a 2-mercaptopbenzothiazole compound  
conforming to the formula



10  
20  
25  
30  
35  
40

wherein  $\text{R}^3$  is selected from hydrogen or from alkyl,  
aryl, or cycloalkyl radicals, or combinations thereof,  
containing from 1 to about 12 carbon atoms per radical,  
and wherein the total of all the carbon atoms in  
all of the  $\text{R}^3$  radicals on the molecule will not exceed  
about 20;

additive (E) is lead naphthenate;

additive (F) is an alkali metal salt of a dinonylnaphthalene sulfonate corresponding to the formula



wherein M is an alkali metal and the  $\text{C}_9\text{H}_{19}$  radicals  
are either branched or unbranched radicals;

additive (G) is octylated diphenylamines corresponding  
to the formula



wherein the  $\text{C}_8\text{H}_{17}$  radical can be either branched or  
unbranched.

References Cited

UNITED STATES PATENTS

|           |         |                 |       |          |
|-----------|---------|-----------------|-------|----------|
| 2,898,301 | 8/1959  | Mayhew et al.   | ----- | 252—51.5 |
| 2,923,738 | 2/1960  | Williams et al. | ----- | 252—51.5 |
| 2,958,665 | 11/1960 | Stefcik et al.  | ----- | 252—51.5 |
| 3,108,070 | 10/1963 | Hartung et al.  | ----- | 252—33.3 |
| 3,112,270 | 11/1963 | Mitacek et al.  | ----- | 252—59   |
| 3,125,530 | 3/1964  | Mayhew et al.   | ----- | 252—51.5 |

DANIEL E. WYMAN, Primary Examiner

I. VAUGHN, Assistant Examiner

U.S. Cl. X.R.

40  
252—33.6, 37.7, 47, 51.5, 59

UNITED STATES PATENT OFFICE  
CERTIFICATE OF CORRECTION

Patent No. 3,539,512 Dated November 10, 1970

Inventor(s) Raymond Rohde et al.

It is certified that error appears in the above-identified patent and that said Letters Patent are hereby corrected as shown below:

Column 4, line 39, "195" should read -- (195 --; line 40, "11.50" should read -- 81.00 --; line 52, "85.0" should read -- 85.8 --. Column 6, the formula appearing at line 35 should read as follows:



Signed and sealed this 2nd day of March 1971.

(SEAL)

Attest:

EDWARD M. FLETCHER, JR.  
Attesting Officer

WILLIAM E. SCHUYLER, JR.  
Commissioner of Patents